

## UNITED STATES PATENT OFFICE

2,334,816

## NONMAGNETIC RING COMPOSITION

Harry L. Frevert and Francis B. Foley, Philadelphia, Pa., assignors to The Midvale Company, Philadelphia, Pa., a corporation of Delaware

No Drawing. Application August 21, 1943,  
Serial No. 499,548

6 Claims. (Cl. 75—128)

In the manufacture of non-magnetic retaining rings it has always been necessary to use a composition of steel containing an amount of alloy, usually nickel, chromium and manganese, such that the iron takes on the gamma, or face-centered cubic type of crystalline form which is non-magnetic and little subject to modification by heat treatment. The strength of such an alloy steel is not materially affected by the process of quenching and tempering in the manner commonly used in the hardening of ordinary steels. Strength, however, is an important attribute of non-magnetic steels and it has been necessary to increase the inherent strength of non-magnetic steels used as retaining rings by deformation at slightly elevated temperatures, a process not so easily carried out with the masses involved as it is in the production of wire and sheet of austenitic steel.

The extent to which the strength and hardness of a metal may be increased by the process of deforming at low temperatures is dependent not only on the degree of deformation and the temperature at which deformation takes place, but also on the thickness of the metal. In heavy masses the effects of deformation tend ordinarily to be confined to the surface layers, whereas in thin material the effects readily penetrate throughout the section. In thick sections it is not unusual to find high tensile strength in the surface metal and very much lower strength in the deep-seated layers of a forging.

Compositions of steel known to respond in a manner to the strengthening effect of deformation at low temperature and to be practically non-magnetic have the following composition range:

| C       | Mn       | Si      | Ni       | Cr      | W       | Mo      |                          |
|---------|----------|---------|----------|---------|---------|---------|--------------------------|
| Percent | Percent  | Percent | Percent  | Percent | Percent | Percent | Balance principally iron |
| 1.0     | 5.0/10.0 | .50     | 8.0/11.0 | 4.0/8.0 | 1       | 1       |                          |

<sup>1</sup> Maximum.

And have the following preferable composition range:

| C       | Mn      | Si      | Ni      | Cr      | Mo      | W       |
|---------|---------|---------|---------|---------|---------|---------|
| Percent | Percent | Percent | Percent | Percent | Percent | Percent |
| .4-.6   | 5-7.5   | .3-.6   | 8.8-10  | 4.5-6.5 | 1-.3    | .1-.6   |

The following are specific examples of compositions within the above ranges:

| 5 |   | C   | Mn   | Si | Ni   | Cr   | W   | Mo  |
|---|---|-----|------|----|------|------|-----|-----|
|   | A | .58 | 5.33 | —  | 9.03 | 5.32 | .15 | .52 |
|   | B | .70 | 5.50 | —  | 9.30 | 4.80 | .10 | .38 |
|   | C | .74 | 5.72 | —  | 9.40 | 5.50 | .10 | .52 |

10 The silicon content is immaterial and may be that common in carbon steel, say not less than about .15% and not over about 1%.

15 By finishing forging such a composition of austenitic steel at temperatures in the neighborhood of 1200° F. a high tensile strength may be produced together with an adequate degree of ductility as measured by the percentage of elongation and of reduction of area of the metal

20 when ruptured under tension stresses. The results produced, however, are frequently of such a nature as to be quite misleading in at least two respects: First, the effects of the deformation at low forging temperature are frequently

25 found to have been confined to the surface metal; and, secondly, the yield strength of the metal is not increased at the same rate as is the tensile strength and does not therefore attain values frequently demanded by the stresses imposed by service conditions. The yield point of the metal is of great importance, since the rings under discussion are usually subject to high speed revolution in service and failure is likely to be disastrous.

30 Not only is it of the utmost importance that the Y. P. should be as high as possible, but it is also of importance that the Y. P. should have a high percentage rate relative to the T. S. A wide spread between T. S. and Y. P. is a defect 35 frequently found in the inner properties of rings deformed at low forging temperature.

40 The undesirable quality above described may be 45 illustrated by actual cases of rings from the heats A, B and C above listed. The properties, absolute and relative, of T. S. and Y. P. exhibited in a surface metal test when finished forged were satisfactory. For example, such a test from heat A showed T. S. 144,000 p. s. i. and Y. P. 114,000 p. s. i. However, test bars taken deeply within the ring showed T. S. 114,000 p. s. i. This test illustrates the great loss of T. S. in deeply seated tensile bars.

45 50 As illustrative of the wide spreads that frequently occur between T. S. and Y. P. may be cited

tests made of material deeply within retaining rings from heats B and C.

|        | T. S.           | Y. P.         | Elong.    | Red. of area |
|--------|-----------------|---------------|-----------|--------------|
|        | P. s. t.        | P. s. t.      | Percent   | Percent      |
| B----- | 150,000/153,750 | 112,000       | 26.0/34.0 | 28.2/34.7    |
| C----- | 130,000/134,000 | 75,000/81,000 | 25/33     | 33.0/39.0    |

These tests illustrate the wide spread between T. S. and Y. P., the percentage of the latter to the former varying from 60 to 74%.

We have found that the addition of .05 to .3% nitrogen to alloys of the above type has profound beneficial effects. Not only does it increase the Y. P. but it enables the high T. S. and Y. P. combination to be attained without having to carry deformation at temperatures as low as have been required heretofore and produces properties that are high throughout the section with little danger of being misled by the appearance of high strength in the exterior of a forging.

As typical examples of improvements effected by addition of nitrogen to the material may be cited tests made with rings of the following compositions:

|        | C   | Mn   | Si  | Ni   | Cr   | Mo  | W   | N <sup>2</sup> added |
|--------|-----|------|-----|------|------|-----|-----|----------------------|
| D----- | .57 | 5.48 | .52 | 9.05 | 4.75 | .15 | .49 | .13                  |
| E----- | .44 | 6.90 | .50 | 9.70 | 5.77 | .28 | .11 | .15                  |

Two rings were made from heat D and two from heat E, the tests being made of material deeply within the ring, with the following results:

|              | T. S.           | Y. P.           | Elong.    | Red. of area |
|--------------|-----------------|-----------------|-----------|--------------|
|              | P. s. t.        | P. s. t.        | Percent   | Percent      |
| D-----       | 142,500/152,000 | 114,000/124,000 | 18.7/26.5 | 22.4/29.1    |
| Average----- | 146,700         | 121,600         | 19.5      | 25.1         |
| D-----       | 145,000/155,000 | 116,500/130,000 | 25.5/33.0 | 26.8/41.3    |
| Average----- | 149,700         | 124,200         | 29.5      | 35.4         |
| E-----       | 121,500         | 97,500          | 43.2      | 52.5         |
| E-----       | 121,500         | 96,500          | 43.2      | 54.9         |

Comparing the tests on B and D, it will be noted that even though B showed a T. S. comparable with (somewhat higher than) D, it showed a much lower Y. P.; the percentage ratios of Y. P. to T. S. being less than 74% for B as contrasted with over 83% for D.

Comparing the tests C and E, whose tensile strengths were considerably lower than the tensile strengths of B and D, it will be noted that while the T. S. of C was higher than that of E, its Y. P. was much lower; the percentage ratios of Y. P. to T. S. being about 60% for C as compared with about 80% for E.

In general it may be stated that in the deep-seated regions of non-nitrogen-bearing rings of the composition specified the Y. P. will vary, with different compositions, from below 60% to less than 75% of the T. S., while with Ni added the Y. S. will in most compositions run substantially over 75% and usually between 78% and 85% of the T. S.

A convenient method of adding the nitrogen is by means of nitrogen-bearing ferro-chromium, although the method of adding the nitrogen is not a determining factor in the result obtained.

5 It should be understood, however, that the percentage of nitrogen shown by analysis of the rings may be considerably less than the amount of nitrogen added. With nitrogen added in percentages from .05 to .3%, the percentage of nitrogen 10 in the final composition will vary from about .03 to .25%; the amounts of the loss varying, roughly, but by no means exactly, in proportion to the amounts of the additions.

What we claim and desire to protect by Letters Patent is:

15 1. A ferrous alloy of low magnetic permeability capable in thick sections of developing, by working at moderately low temperatures, a high tensile strength, a high yield point and a yield point which is high relative to the tensile strength, deeply within, as well as near the surface, said alloy having a composition comprising carbon .05 to 1%, manganese 5 to 10%, silicon .15 to 1%, nickel 8 to 11%, chromium 4 to 8%, metals of the 20 group comprising molybdenum and tungsten .25 to 3%, nitrogen .03% to .25%, and substantially all the remainder iron with its normal impurities, and characterized by having a yield point substantially exceeding 75% of its tensile strength.

25 2. A ferrous alloy of low magnetic permeability capable in thick sections of developing, by working at moderately low temperatures, a high tensile strength, a high yield point and a yield point which is high relative to the tensile strength, 30 deeply within, as well as near the surface, said alloy having a composition comprising carbon .05 to 1%, manganese 5 to 10%, silicon .15 to 1%, nickel 8 to 11%, chromium 4 to 8%, metals of the group comprising molybdenum and tungsten .25 to 3%, nitrogen .03 to .25%, and substantially all the remainder iron with its normal impurities, and characterized by having a yield point between about 78 and 85% of the tensile strength.

35 3. As a new article of manufacture, a non-magnetic ring composed of the ferrous alloy specified in claim 1 and having throughout its entire mass the yield point—tensile strength ratio specified in claim 1.

40 4. As a new article of manufacture, a non-magnetic ring composed of the ferrous alloy specified in claim 2 and having in regions thereof most distant from the surface a yield point substantially exceeding 75% of its tensile strength.

45 5. As a new article of manufacture, a non-magnetic ring composed of the ferrous alloy specified in claim 2 and having throughout its entire mass the yield point—tensile strength ratio specified in claim 2.

60 6. As a new article of manufacture, a non-magnetic ring composed of the ferrous alloy specified in claim 2 and having in regions thereof most distant from the surface a yield point between about 78 and 85% of the tensile strength.

65

HARRY L. FREVERT.  
FRANCIS B. FOLEY.